

## UNITED STATES PATENT OFFICE

1,927,927

ADHESIVE AND PROCESS OF MAKING  
SAME

Henry V. Dunham, Bainbridge, N. Y.

No Drawing. Application July 10, 1929  
Serial No. 377,334

5 Claims. (Cl. 87—17)

The present invention relates to improving adhesives or glues of the kind used for gluing up plywood, and for wood-working generally. In accordance with the present invention it is found 5 that by employing a small percentage of pine oil (preferably steam distilled pine oil, first added to or preferably emulsified in the water with which the dry glue base is mixed up) the adhesive is somewhat improved in a number of respects, the principal advantage being that it gives a smoother working glue and is less likely to foam. The invention is applicable particularly to the wood-working glues containing casein or seed-meal or a mixture of these, together with lime (preferably hydrated lime, or magnesium oxide or hydroxide, or other alkaline earth base), and containing an alkaline reacting salt of an alkali metal such as sodium carbonate, sodium phosphate and similar salt, which 10 can react with the lime in the presence of water to produce caustic alkali which at once reacts with the protein of the seed-meal or with the casein or with both, to constitute a solution of alkali casein or alkali protein.

Without restricting the invention to specific examples of the glue base, the following are given as satisfactory examples:—

## Example 1

30 Peanut flour or cotton-seed flour 67 parts, calcium hydroxide 18 parts, sodium carbonate 7 parts, trisodium phosphate 4 parts, sodium fluoride 4 parts.

## Example 2

35 I mix together 70 parts of commercial dry casein, 10 parts of tri-sodium phosphate, 20 parts of slaked lime (calcium hydroxide) and 3 parts of dry sodium fluoride, mix together and pass 40 through a 30 mesh screen.

## Example 3

Linseed meal or peanut meal 30 parts, dry casein (40 mesh) 26 parts, hydrated lime 19 parts, 45 sodium carbonate 6 parts, tri-sodium phosphate 5 parts, sodium fluoride 3 parts.

The vegetable seed-meals referred to in the above examples may constitute the residue left from expressing the oil, or this residue may be 50 further extracted with oil solvents, to remove most of the oil. Ordinarily it is preferable to leave about 5 to 7 per cent of the oil in the meal. The press cakes are in all cases preferably ground to pass through a mesh of 30 to 40. 55 Where peanut flour is referred to this may be

made from the whole peanut kernels (preferably unroasted) or from the kernels after removal of a portion of the red skins. A small amount of the peanut shells may be left in if desired, or may be added to the dry glue base, after being 60 finely pulverized to pass through a 50 or 60 mesh screen.

The above examples constitute suitable dry glue bases for use in connection with the present invention, and are not claimed as such in the 65 present case, as a part of the present invention.

Shortly before the time of use of the glue, it is made into a liquid glue, by being mixed up with two to three times its own weight of water containing a small percentage of pine oil. It is 70 not necessary to first emulsify the oil, since as the casein dissolves, it forms an excellent emulsifying agent for the pine oil. By the time the glue has become thoroughly incorporated with the water (or "dissolved" as this is usually called 75 in the art) the pine oil will be found to be thoroughly emulsified.

Or the pine oil is first emulsified in the water, by the use of a suitable emulsifying agent. Sulfonated castor oil or sulfonated castor oil soap, 80 or other sulfonated vegetable oil or sulfonated animal oil or sulfonated mineral oil, or the soaps of these can be used as emulsifying agents. Stable emulsions of rosin soap with pine oil, now known on the market can likewise be used. A 85 pasty material made up of about equal parts of concentrated laundry soap solution with pine oil, likewise could be used as the source of the pine oil. I prefer to use straight pine oil without added emulsifying agents. 90

In preparing the glue from the glue base, the pine oil (or say a mixture of two parts of steam distilled pine oil with one part of sulfonated castor oil) is preferably first added to the bulk of water which is to be used. 95

The mixture may then be stirred for a few minutes or not, as desired. To this the dry glue base is then added in the same manner as it is ordinarily added to water, and in the same proportion. One part of the dry base will require 100 from two to three parts of water, about two and a half parts being a fair average. The amount of the pine oil used may be equal to about 1 to 5 per cent of the dry glue base (or about 0.4% to 2.5% of the amount of water). 105

Ordinarily it is advisable to mix glues of the kind referred to above, with cold water, say at 60° F. However, in many places the workmen prefer to use simply tap water, at whatever temperature it may be found. Thus in the South, 110

- in summer time, the mixing water might be at 90° F. and the atmospheric temperature at 100° F. Under these conditions the glue might foam considerably. The use of say 3% or 4% of pine oil simply dumped into the mixing water in the kettle before adding the glue base (or simultaneously with adding the glue base, but separately therefrom) will wholly overcome the foaminess under these conditions. Glue bases 5 that are old, i. e. have been mixed up for six months or a year) also have more tendency to foaminess than "fresh" material, and here the foaminess can be abated by adding pine oil, as described herein.
- 10 15 The following example is given, concerning the mixing operation, although it will be understood that the invention is not restricted to this specific example.

20

*Example 4*

- To 200 parts of water (preferably cold) is added 2 parts of steam distilled pine oil. 100 parts of the dry glue base as given in Example 2 above referred to, are then added and the stirring 25 continued for 15 minutes, or so or until the mixture is sufficiently uniform and has a sufficiently smooth flow for use on a glue spreading machine used in making up plywood.

If the mixing water is rather warm and if the glue is rather old, 5 parts of the pine oil might be used in this example. I make no claim herein to abatement of foam by adding the pine oil to the dry glue base. It has been common practice for many years, to "oil" casein which is to be used in making a dry glue base. This step, as commonly practiced, has been to simply mix a little oil, (e. g. 1 to 3%) with the dry ground casein. Pine oil so used on the casein or on the dry glue base, does not have the effect of preventing foaminess of the liquid glue, to the production of which effect the present invention is particularly directed.

What is claimed is:—

1. A process which comprises mixing a dry glue base comprising an alkali-soluble proteinaceous material, an alkaline earth base and an alkaline compound of an alkali metal with about two to three times its own weight of water containing a small amount of pine oil separately admixed therewith. 80

2. A process which comprises mixing a dry glue base comprising an alkali-soluble proteinaceous material, an alkaline earth base and an alkaline compound of an alkali metal with about two to three times its own weight of an aqueous emulsion of pine oil and a sulfonated oil material. 85

3. In the mixing of water with dry glue base comprising an alkali-soluble proteinaceous material, an alkaline earth base and an alkaline compound of an alkali metal and which shows considerable tendency to foam, the step of adding about 1 to 5% of pine oil to the water, such step being separate from the addition of the glue base thereto. 90

4. In the art of mixing with water a stale dry glue base which has a tendency to foam, the 100 said base containing casein, alkaline earth hydroxide and alkali metal compounds capable of acting as casein solvents, the herein described step of adding to the water a small percentage of pine oil separately from the glue base. 105

5. In the art of mixing with water a stale composite dry glue base which has a tendency to foam, said base containing casein, seed meal high in protein, alkaline earth hydroxide and alkali metal salts serving as solvents for the 110 casein and meal proteins, the herein described step of mixing with the water a small percentage of pine oil separately from the glue base, for the purpose of preventing foam. 115

HENRY V. DUNHAM.

45

120

50

125

55

130

60

135

65

140

70

145